

Jan. 8, 1946.

R. G. CHOLLAR

2,392,521

POROUS RESILIENT PRINTING PLATE

Original Filed Feb. 12, 1942

FIG. 1



FIG. 2



Robert G. Chollar  
Inventor

By *Earl Beust*  
His Attorney

## UNITED STATES PATENT OFFICE

2,392,521

## POROUS RESILIENT PRINTING PLATE

Robert G. Chollar, Dayton, Ohio, assignor to The National Cash Register Company, Dayton, Ohio, a corporation of Maryland

Original application February 12, 1942, Serial No. 430,661. Divided and this application April 1, 1943, Serial No. 481,419

9 Claims. (Cl. 101—327)

This application is a division of my co-pending application Serial No. 430,661, filed February 12, 1942, now Patent No. 2,349,613, issued May 23, 1944.

This invention relates to resilient micro-porous printing plates and more particularly relates to such micro-porous resilient printing plates in which the resilient body acts as a reservoir and as a conductor for ink which is supplied to the type face through the pores.

It is known in the art of printing that porous printing members may be made of various materials more or less hard in structure to be used to absorb and conduct ink to a printing surface inscribed thereon. These porous substances have been non-resilient, so that printing qualities characteristic of a resilient surface equivalent to that of rubber could not be obtained. Heretofore, an ink-resistant porous printing plate of sufficient strength for commercial use and of the fine surface porosity necessary to give even printing has not been produced.

This invention relates to a printing member or plate made of porous rubber or rubber-like material either of a single layer or of laminated structure, as will be described, said porous rubber and the process for making it being described in my co-pending application for United States Letters Patent Serial No. 427,326, filed on the nineteenth day of January, 1942, now Patent No. 2,353,877, issued on July 18, 1944.

The printing member which is the subject of this invention is a consolidated laminated member, the main body of which is coarsely micro-porous and the printing surface of which is finely micro-porous, the two layers being bonded together in such a fashion that ink passes readily from one layer to another. Said coarser layer of the laminated structure is re-supplied with ink by means of a wick-like backing, which backing may be of porous metal, of woven fabric, of felted fiber, or of any other capillary conducting substance.

Therefore, the principal object of this invention is to provide a resilient micro-porous printing member.

Another object of the invention is to provide a resilient micro-porous printing member having a surface layer for printing which is more finely micro-porous than the principal body of the member.

Another object of the invention is to provide a resilient porous printing member with a non-resilient porous backing.

Another object of the invention is to provide

a printing member having a printing surface made of micro-porous rubber-like material which is supplied with ink through a coarsely micro-porous body structure by means of a wick-like structure.

Another object of the invention is to provide a process for making the aforesaid objects.

With these and incidental objects in view, the invention includes certain novel features of construction and combinations of parts, the essential elements of which are set forth in appended claims and a preferred form or embodiment of which is hereinafter described with reference to the drawing which accompanies and forms a part 15 of this specification.

In said drawing:

Fig. 1 is a cross-sectional view, in diagrammatic form, of the novel laminated resilient porous structure and means for supplying ink thereto.

Fig. 2 is a diagrammatical perspective view, partly broken away, of a typical porous resilient laminated printing plate and of the inking means therefor.

## General description

The laminated printing member is made up of a finely porous layer 10 formed of particles of raw material passing a screen of less than 325 mesh to the inch in size, and of another layer 11, which is a coarser backing layer made up of particles of raw material passing a screen of from less than 25 to 100 mesh to the inch in size, as will be described. The two layers merge into one another at their juncture in such a fashion that the pores of one layer intercommunicate with the pores of the adjacent layer, so that whatever fluid recording material is contained in the layer 11 is transmitted by capillary action to the layer 10. The porous layer 10, which forms the printing surface, is made with fine pores because it makes a more even impression, as the individual pores therein are not discernible by reason of the mark deposited from the pore openings on recording material.

A method of making the porous rubber, although adequately described in my Patent No. 2,353,877, to which reference has been made, will be summarized briefly herein.

Rubber or synthetic rubber finely comminuted to the proper mesh size, said synthetic rubber being preferably of the butadiene co-polymer type, containing ordinary vulcanizing ingredients, is mixed 55 parts by volume with 45 parts by volume of a finely comminuted filler. One such mixture is made of particles approximately less

than the 325 mesh size, and one mixture is made with particles approximately less than the 25 to 100 mesh size. The finer mix is made into a fluid mass, like a rubber cement, by the addition of a volatile solvent such as methyl-ethyl-ketone and is applied to one surface of a  $\frac{1}{1000}$ -inch thick water-soluble poly-vinyl alcohol sheet, said coating being made thick enough so that when dry it is approximately  $\frac{2}{1000}$  of an inch in thickness as a maximum. The poly-vinyl alcohol sheet with the coating thereon is placed in a die against a matrix of the printing surface to be formed, which matrix may be of Bakelite or other material that will withstand pressure and heat and will not adhere to the poly-vinyl alcohol. The uncoated side of the poly-vinyl alcohol sheet is placed next to the matrix. On top of this coating, preferably when dry, is placed the powder mix of the coarser variety so as to give the coarser layer, when molded, a maximum thickness of between  $\frac{3}{1000}$  of an inch and  $\frac{12}{1000}$  of an inch. The whole mass in the mold is compressed between the matrix and a ram with a pressure of between 250 pounds to the square inch and 6000 pounds to the square inch, as the material requires, and then is vulcanized. The butadiene co-polymers require a temperature of about 307 degrees Fahrenheit for vulcanizing, which may be applied either in or out of the mold. The molded plate is removed from the mold, and the filler, which preferably is sodium nitrate, is dissolved out by washing in a solvent which has no effect upon the resilient material used. Sodium nitrate may be washed out with hot water containing a wetting agent, such as soap or one of the aliphatic penetrants. Other fillers suggested are powdered metals, including powdered zinc; sodium carbonate; ammonium sulphate; or powdered water-soluble poly-vinyl alcohol.

The sodium nitrate may be washed out of a printing plate one-tenth of an inch thick in about two hours, if it is agitated in hot water. The water in the pores after a washing process is preferably replaced with ink by immersing the plate in ink above the boiling point of water, thus preventing possible adhesions of the pore surfaces. For the zinc, the carbonates, and the nitrates, acids may also be used, hydrochloric acid and dilute nitric acid being suggested. With the percentage of ingredients named, the porosity of the printing plate as a unit is about 45% by volume and will absorb by volume about 45% ink. A dye ink of the oleic acid vehicle type is suitable for use with the particular synthetic rubber mentioned.

The back of the printing plate may have bonded thereto by molding it with the rubber mix, as a third and last layer in the mold, fabric, felt, ribbon, blotting paper, or a porous metal plate 12 to act as a strengthening support for the porous rubber and as a means to re-ink the porous rubber by means of a wick 13 inserted therein.

It is to be understood that the particular materials suggested are not to limit the scope of the invention. The particular size of the particles in the mix are specified as being best adapted for dye inks having an oil base. The butadiene co-polymers are resistant to corrosion by such inks. The sodium nitrate is preferred as a filler, as it may be washed out of the molded material with hot water, which will also dissolve any of the poly-vinyl alcohol sheet that cannot be removed by peeling. For other inks, for thicker plates, or for different molding temperatures, the ingredients must be selected on the basis of their

suitability. It is within the intended scope of this invention to make such laminated plates with more than two layers.

In Fig. 1, the portion 14 represents a character 5 molded in the web, the cross-sectioned portion 15 showing the effect on the two layers after being forced into the matrix of the character.

The use of water-soluble poly-vinyl alcohol in the process described makes it possible to wash 10 the poly-vinyl alcohol sheet off the molded mass as the filler is washed out to make the rubber porous.

The printing plate described is very compressible, and printing made from such a plate should 15 be very light contact, which can be assured by surrounding the printing plate by non-resilient stops, preventing compression of the printing plate by contact with the record material. The supply of ink available at the type surface is so 20 copious that a light and fast contact is all that is necessary to make a well-defined impression. Therefore, the printing plate, not being subjected to severe hammering and pressure, will last indefinitely as compared with ordinary printing plates, even though the porous structure is rather 25 fragile as compared with solid printing plates.

It is obvious that the laminated structure shown may be used for filtering or for separating 30 liquids or for separating solid material either in gases or in liquids, or may be used for wicks for various purposes. The laminated structure for printing plates is, however, most important if fine printing is to be combined with high ink 35 capacity and rapid recovery of the printing qualities after an impression. The preferred embodiment described produces a printing plate that will accommodate itself to impressions less than a second apart for extended periods.

While the product made in accordance with 40 the process described herein is admirably adapted to fulfill the objects primarily stated, it is to be understood that the invention is directed particularly to the laminated structure. It is not intended to confine the invention to the preferred 45 form or embodiment herein disclosed, for it is susceptible of embodiment in various forms by varying ingredients and processing steps, all coming within the scope of the claims which follow.

50 What is claimed is:

1. A printing type consisting of a web of two joined layers of vulcanized micro-porous rubber saturated with ink, one of said layers being of finer porous structure than the other of said layers, the layer of finer porous structure having a printing surface consisting of printing characters, and the pores of each layer being interconnected and the pores of one layer connected to the pores of the other layer to provide means for the ink to pass from one layer to the other and to the printing surface by capillary action.

2. An ink-saturated micro-porous rubber printing type, consisting of joined layers of said micro-porous rubber, the pores in each layer being interconnected and the pores of the different layers being interconnecting, the pores of a layer being approximately of uniform size but the pores of the different layers being ununiform as to size, the printing surface of the type being formed 65 on the surface of the layer having the smaller pores.

3. A printing type made of a sheet of micro-porous rubber, the pores on the printing surface being smaller than the pores in the back of said 70 sheet, the larger pores acting as a reservoir and

the smaller pores acting to control the flow of ink to the printing surface.

4. A laminated printing type made of micro-porous rubber, formed of a layer of finely porous rubber having a surface thereof formed into a printing surface, and a layer of micro-porous rubber relatively coarse joined to said layer of finely porous rubber, the intercommunication of the pores from one layer to another being maintained.

5. A printing type formed of micro-porous rubber, having a printing surface consisting of a film of very fine micro-porous rubber, which pores are communicative with the pores of the rest of the body, the pores of the said rest of the body being relatively coarser than the film.

6. A printing member consisting of a laminated micro-porous rubber structure, one of said laminations having smaller voids in the pore structure than the other, said one lamination being formed into relief to make printing characters, and said finer laminated layer and said

other laminated layer being formed together, and a porous backing for said printing member.

7. A laminated structure of porous material forming a printing type consisting of a backing layer of relatively strong porous material, a middle layer consisting of porous and resilient rubber, and a printing layer consisting of fine micro-porous resilient rubber, all of said members being bonded together and having their pores inter-

10 communicating and saturated with ink.

8. A printing type made of a layer of vulcanized, resilient micro-porous butadiene co-polymer rubber backed by a porous structure of relatively greater strength, said rubber layer having printing characters therein.

9. A printing type made of a layer of vulcanized resilient porous butadiene co-polymer rubber overlaid with a layer of the same material having a finer pore structure, and printing characters in said latter layer.

ROBERT G. CHOLLAR.